

Sept. 24, 1929.

W. M. CHACE

1,729,245

THERMOSTATIC ELEMENT

Filed Dec. 19, 1927



INVENTOR.

WILLIAM M. CHACE

BY

Charles E. Wilson  
ATTORNEY.

## UNITED STATES PATENT OFFICE

WILLIAM M. CHACE, OF DETROIT, MICHIGAN; ADELBERT H. LINDLEY, ARTHUR COOPER, AND HILMA B. CHACE, EXECUTORS OF SAID WILLIAM M. CHACE, DECEASED, ASSIGNEES TO W. M. CHACE VALVE COMPANY, OF DETROIT, MICHIGAN, A CORPORATION OF MICHIGAN

## THERMOSTATIC ELEMENT

Application filed December 18, 1927. Serial No. 241,275.

This invention relates to bimetallic elements such as are ordinarily used in various positions where it is subjected to variation in temperature and to perform work by its consequent transient deformation as in the making and breaking of the electric circuit or control of various devices, and the purpose of the invention is to secure a bimetallic element in which the greatest movement is within 5 in a temperature range of from about 400 to 700 degrees F., and that is less responsive to temperature change below or above such temperature range and further one that may be subjected to high temperature without 10 permanent deformation.

The accompanying drawing is a diagram illustrating the expansion curve of my improved thermostatic couple.

Various efforts have been made in the past 20 to secure a bimetallic element having such characteristics the purpose being to secure a device that is very rapid in movement through the temperature range in which its movement is to be utilized and has little or 25 no movement at temperatures outside of said range. For instance, in an electric iron, a bimetallic disk is used to make and break the circuit but if the disk is made of two elements liable to permanent deformation at 30 temperatures in the neighborhood of 500 degrees F., the device is of short life and therefore not practical to use at such temperatures, and again for instance in a thermostatic spark plug, one of the electrodes being made 35 of a bimetallic element which is subject to the heat developed in the cylinder of an internal combustion engine, it is not desirable for the thermostatic electrode to materially move from close association with the other 40 fixed electrode until it has attained a temperature above 400 degrees F., and must not be subject to permanent deformation at temperatures around 2000 degrees F., in continued operation of the engine.

45 The commonly known invar and brass bimetallic element is not efficient for this purpose although sensitive at temperatures below 500 degrees F., and it is also known that certain nickel steels having a greater difference of expansion than the invar-brass

combination but the known composition of nickel steels such for instance as described in the U. S. patent to Miller, No. 1,604,064 or my own Patent No. 1,642,485 are sufficiently rapid in movement at temperatures 55 above 500 degrees F. While such blades are effective for some purposes they are ineffective where the movement is desired to be as constant per degree of temperature change 60 500 to 700 degrees F., as they are from 400 to 500 degrees F.

In the research and experimental work to find a composition of elements for the expansion side of a bimetallic blade or plate, I have discovered that the nickel content may 65 be reduced below that disclosed in either of the U. S. patents above mentioned and the chromium and copper increased relative to the percentage thereof disclosed in my said former patent and still secure a composition 70 of practically the same coefficient of expansion and secure movement through a higher range of temperature than has heretofore been attained. This composition is welded to an element containing approximately 75 forty per cent of nickel and being more sensitive to temperature change than invar, counteracts the tendency of the expansion element to cause movement or restricting such movement until the desired 80 temperature is attained whereupon the movement is rapid through the described temperature range. A bimetallic element having the described characteristics may be formed of two plates, blades, or sheets of metal of the 85 following respective compositions welded together. The neutral side preferably consists of—

|         |   |       |    |
|---------|---|-------|----|
| Carbon  | — | .35   | 90 |
| Silicon | — | 2.00  |    |
| Nickel  | — | 40.00 |    |
| Iron    | — | 57.65 |    |

and the expansion side consists of—

|              |   |          |       |     |
|--------------|---|----------|-------|-----|
| Carbon       | — | .25 to   | .35   | 95  |
| Silicon      | — | 1.75 to  | 2.00  |     |
| Chromium     | — | 13.25 to | 14.00 |     |
| Nickel       | — | 2.50 to  | 3.50  |     |
| Copper       | — | 5.00 to  | 7.00  |     |
| Wrought iron | — | 77.25 to | 73.15 | 100 |

The elements above enumerated are the usual named elements of commerce and the iron utilized (particularly in the expansion element) is preferably what is known to the trade as "Swedish iron" because of its purity and containing a trace of copper.

The elements comprising the expansion side are given to indicate the present known permissible variation in quantity of each.

10 This bimetallic element has the characteristics as is shown in the accompanying diagram by the heavy line. The horizontal lines of the diagram represent inches of movement while the vertical lines are the temperature lines under which the movement takes place, of bimetallic strips of a size .048 inches thick by 1/2 inch wide by 5 1/8 inches long. It will be apparent from the diagram that, with such a strip held stationary at one end, the movement at the opposite or free end through temperature of 350 degrees F., is approximately 4/10 of an inch and for each 100 degrees of change in temperature from 350 to 700 degrees F., and that the movement is practically 20 4/10 of an inch and therefore is practically constant for each 100 degrees change up to 700 degrees, and that from 700 to 800 degrees the movement is only about 1/10 of an inch. Thus, by use of my new composition for the 30 expansion side in conjunction with an element containing approximately 40 per cent of nickel I obtain a bimetallic element that has very little movement below 300 degrees F., or above 700 degrees F., and that the 35 movement is very rapid and practically constant for each degree of change in a temperature range of from about 350 to 700 degrees F.

Due to the fact that movement in the bimetallic strip or plate is caused by reason of the difference in coefficient of expansion of the two elements forming the same, I believe the peculiar movement curve of my new element is secured by reason of the fact that what I 45 have termed the "neutral" side does not have a fixed coefficient of expansion throughout the temperature range described but on the contrary, expands to a degree approximating that of the expansion side up to 350 degrees 50 F., and from 350 to about 700 degrees has very little or no expansion and above the said temperature expands on to a degree more closely approximating that of the expansion side. That this is strictly the fact, however, 55 I am unable to determine inasmuch as the expansion side of the element also may have a coefficient of expansion varying under the different degrees of heat to which it is subjected.

60 A bimetallic element of two plates or blades of the respective compositions mentioned is capable of withstanding temperatures as high as 2000 degrees F., without permanent deformation or loss of elasticity, and the preferable method of securing the two parts together is 65 by first welding with a flux between the plates

and then rolling the same while hot. Subsequent to the rolling operation, the bimetallic sheet may be cut into blades, strips or plates or other forms depending upon the purpose for or the device with which the element is 70 to be utilized.

Having thus fully described my invention, what I claim and desire to secure by Letters Patent of the United States is—

1. A bimetallic thermometer consisting of 75 two metal parts welded together, one of said parts consisting of the following elements approximately of the stated percentage—viz,

|         |       |    |
|---------|-------|----|
| Carbon  | 35    | 80 |
| Silicon | 2.00  |    |
| Nickel  | 40.00 |    |
| Iron    | 57.65 |    |

and the other part consisting of the following 85 elements approximately of the percentage stated—viz,

|              |       |    |
|--------------|-------|----|
| Carbon       | 25    |    |
| Silicon      | 1.75  | 90 |
| Chromium     | 13.25 |    |
| Nickel       | 2.50  |    |
| Copper       | 5.00  |    |
| Wrought iron | 77.25 |    |

2. A bimetallic thermometer capable of being subjected to temperatures as high as 2000 degrees F., without permanent deformation consisting of two metal parts welded together in a unitary structure and characterized by 100 having pronounced dissimilar thermal characteristics within a specific temperature range, one of the parts consisting of the following ingredients substantially in the percentage stated—

|         |       |     |
|---------|-------|-----|
| Carbon  | 35    |     |
| Silicon | 2.00  |     |
| Nickel  | 40.00 |     |
| Iron    | 57.65 | 110 |

and the other consisting of the following ingredients within the specified percentage range—namely,

|              |                |     |
|--------------|----------------|-----|
| Carbon       | 25 to .35      |     |
| Silicon      | 1.75 to 2.00   |     |
| Chromium     | 13.25 to 14.00 |     |
| Nickel       | 2.50 to 3.50   |     |
| Copper       | 5.00 to 7.00   |     |
| Wrought iron | 77.25 to 73.15 | 120 |

3. A thermostatic couple consisting of two metal parts of dissimilar thermal characteristics secured together in a manner to provide a unitary structure in which the thermal characteristics of one oppose or restrict that of the other, the element of low coefficient of expansion being a nickel steel alloy having a nickel content of approximately forty per cent and the element of higher coefficient of 130

expansion being formed of the following ingredients.—

|                       |       |       |    |       |
|-----------------------|-------|-------|----|-------|
| Carbon                | ----- | .25   | to | .35   |
| Silicon               | ----- | 1.75  | to | 2.00  |
| <sup>5</sup> Chromium | ----- | 13.25 | to | 14.00 |
| Nickel                | ----- | 2.50  | to | 3.50  |
| Copper                | ----- | 5.00  | to | 7.00  |
| Wrought iron          | ----- | 77.25 | to | 73.15 |

10 4. A bimetallic thermometer consisting of two nickel steel elements secured together to form a unitary structure, one of the elements containing approximately 40 per cent of nickel and the other containing approximately 14 per cent of nickel and approximately 14 per cent of chromium, the structure being characterized by movement practically constant per degree of temperature change from approximately 350 to 700 degrees F., and being capable of withstanding temperatures as high as 2000 degrees F., without permanent deformation.

15 In testimony whereof I sign this specification.

20 25 WILLIAM M. CHACE.

30

35

40

45

50

55

60

65